

## UNITED STATES PATENT OFFICE

2,600,788

## HALOGEN-SUBSTITUTED PYRAZOLONE COUPLERS FOR COLOR PHOTOGRAPHY

Anthony Loria, Arnold Weissberger, and Paul W. Vittum, Rochester, N. Y., assignors to Eastman Kodak Company, Rochester, N. Y., a corporation of New Jersey

No Drawing. Application June 7, 1949,  
Serial No. 97,701

10 Claims. (Cl. 95—6)

1

This invention relates to photography and particularly to compounds which form dyes on coupling with the developing agent to produce colored images.

It is known that colored photographic images may be formed by using a developer which produces a colored image on development. The colored compound thus formed is deposited adjacent the silver grains of the silver image during development. It is also known that a colored image may be formed by adding to said developer solution or by incorporating in the silver halide emulsion before or after exposure a compound which couples during development with the oxidation product of the developing agent and which forms a colored compound which is likewise deposited adjacent the silver grains of the silver image during development. Such a compound which is employed in conjunction with a developing agent for the silver and which couples with the oxidation product of the developing agent during development is referred to herein as a coupling compound or coupler.

The use of various pyrazolone derivatives for the production of the magenta image in three-color photography is well-known and the use of 1-phenyl-3-acylamino-5-pyrazolones for this purpose is described in Porter and Weissberger U. S. Patent 2,369,489. One of the disadvantages of these couplers is that when the coupler is incorporated in the sensitive emulsion layer, the residual couplers which remain after formation of the dye image is not so stable as is desired and causes discoloration of the final picture. A further disadvantage is that the magenta dye formed from the couplers absorbs more blue light than is desired.

It is therefore an object of the present invention to provide a novel class of couplers for forming the magenta dye image in color photography. A further object is to provide couplers which have improved stability to light and heat when incorporated in the emulsion layer. A still further object is to provide a class of couplers for forming magenta dyes which absorb less blue light than similar couplers and which have a maximum absorption shifted towards the longer wave lengths. Other objects will appear from the following description of our invention.

These objects are accomplished by developing an exposed silver halide emulsion layer with a primary aromatic amino developing agent in the presence of a 1-phenyl-3-acylamino-5-pyrazolone coupler compound having at least two halogen substituents on the 1-phenyl radical. The com-

pounds which we propose to use have the following structural formula:



where  $X$  is halogen, such as chlorine or bromine,  $n$  is two or more and  $COR$  is an acyl radical such as benzoyl, phenyl acetyl, etc. Compounds having the above formula, in which  $X_n$  represents three chlorine substituents are especially valuable for use as couplers according to our invention.

The following compounds illustrate the couplers which may be used according to our invention.

1.



1-(2',4',6'-tribromophenyl)-3-benzamido-5-pyrazolone

2.



1-(2',4',6'-trichlorophenyl)-3-benzamido-5-pyrazolone

3.



1-(2',4',6'-trichlorophenyl)-3-phenylacetamido-5-pyrazolone

4.



1-(2',4',6'-tribromophenyl)-3-phenylacetamido-5-pyrazolone

5.



1-(2',4'-dichlorophenyl)-3-[3''-(2''',4''',di-tert. amyl-phenoxyacetamido)-benzamido]-5-pyrazolone

3



1-(2',5'-dichlorophenyl)-3-[3''-(2'',4''-di-tert. amylphenoxyacetamido)-benzamido]-5-pyrazolone



1-(2',4',6'-trichlorophenyl)-3-[3''-(2'',4''-di-tert. amylphenoxyacetamido)-benzamido]-5-pyrazolone



1-(2',4',6'-tribromophenyl)-3-[3''-(2'',4''-di-tert. amylphenoxyacetamido)-benzamido]-5-pyrazolone



1-(2',4',6'-trichlorophenyl)-3-[β-2''',4''-di-tert. amylphenoxy)-propionamido]-5-pyrazolone



1-(2',4',6'-tribromophenyl)-3-[β-2''',4''-di-tert. amylphenoxy)-propionamido]-5-pyrazolone



1-(2',5'-dichloro)-3-[3''-(4''-tert. amylphenoxy)-benzamido]-5-pyrazolone



1-(2',4',6'-tribromophenyl)-3-[3''-(4''-tert. amylphenoxy)-benzamido]-5-pyrazolone

The compounds of our invention are prepared in general by condensing a dihalo or trihalo aryl hydrazine with ethyl-β-ethoxy-β-imino propionate to form an ethyl-β-(p-haloaryl) hydrazine-β-imino propionate and ring closure of the latter with sodium ethoxide. The imino compound is acylated in the usual manner to form the acylamino pyrazolone.

Compound 1 was prepared as follows:

2,4,6-tribromaniline (Beilstein 12, 663) was diazotized and the cold solution of diazonium salt was added to a cold sodium sulfite solution. The mixture was warmed to 60° C. for 30 minutes and was then esterified with concentrated hydrochloric acid. The reaction mixture was then heated overnight on the steam bath. The 2,4,6-tribromophenylhydrazine hydrochloride was obtained by adding concentrated hydrochloric acid to the hot solution. The hydrochloride was converted

4

to the free base and was added to boiling chlorobenzene, then ethyl-β-ethoxy-β-imino propionate was added and a small amount of glacial acetic acid was added as a catalyst. The mixture was refluxed for five minutes and was then cooled overnight at 0 to 5° C. The crystals of the hydrazine imino propionate were filtered off and washed with cold chlorobenzene and petroleum ether.

10. A solution of sodium ethoxide was prepared from sodium and alcohol and to this was added the ethyl-(2,4,6-tribromophenyl) hydrazine-β-imino propionate prepared above. The mixture was refluxed for 15 to 20 minutes, cooled to 50° C., diluted with water and esterified with glacial acetic acid. 1-(2',4',6'-tribromophenyl)-3-amino-5-pyrazolone separated as a thick, creamy slurry and this mixture was cooled, filtered and the product washed with water and dried at 20 100° C.

The 1-(2',4',6'-tribromophenyl)-3-amino-5-pyrazolone was dissolved in dry pyridine and two moles of benzoyl chloride were added. The mixture was heated for ten minutes on a steam bath, then cooled to room temperature and diluted with water. The product which separated was the dibenzoyl derivative. The dibenzoyl derivative was saponified in alcoholic potassium hydroxide and the solution was filtered and acidified with acetic acid. The 1-(2',4',6'-tribromophenyl)-3-benzamido-5-pyrazolone separated as a solid and was filtered, washed with water and dried and found to have a melting point of 274-276° C.

35. Compound 2 was prepared in the same manner as compound 1 using 2,4,6-trichloroaniline (Beilstein 12, 627) instead of 2,4,6-tribromaniline.

Compound 3 was prepared in the same manner as compound 2, using phenylacetyl chloride 40 in place of benzoyl chloride.

Compound 4 was prepared in the same manner as compound 1, using phenylacetyl chloride in place of benzoyl chloride.

Compound 5 was prepared as follows:

45. 50 grams of 1-(2',4'-dichlorophenyl)-3-amino-5-pyrazolone, prepared as in the preparation of compound 1, using 2,4-dichloroaniline in place of 2,4,6-tribromaniline was placed in a round-bottomed flask together with 625 cc. of glacial acetic acid and 93 grams of m-nitrobenzoyl chloride.

The mixture was heated to boiling and refluxed for 30 minutes. A clear solution was formed but the product began to separate while still hot. The reaction mixture was cooled to room temperature, 55 filtered, washed with 500 cc. of ethyl alcohol and 500 cc. of ether and dried at 100° C. This formed the diacyl derivative which was sifted, suspended in 70% ethyl alcohol and heated to 70° C. and 40% caustic solution was stirred into the mixture.

60. The stirring was continued vigorously for sixty seconds and the mixture acidified with glacial acetic acid. The monoacyl product separated at once and the slurry was stirred and cooled to room temperature. The product was filtered, 65 washed with 200 cc. of ethyl alcohol, and 200 cc. of ether and dried at 100° C. This formed the m-nitrobenzamido derivative and 53 grams of this derivative was placed in a round-bottom flask with 1325 cc. of 90% acetic acid. The mixture

70 was heated to boiling and 53 grams of iron powder were added. The charge was refluxed for fifteen minutes or until all of the nitro compound had dissolved. The solution was then filtered and stirred into two liters of boiling water. This mixture was heated to boiling, cooled to room tem-

perature and filtered. The 1-(2',4'-dichlorophenyl)-3-(3'-aminobenzamido)-5-pyrazolone was washed with 200 cc. of ethyl alcohol, then with 200 cc. of ether and dried at 100° C. This product was then reacted with 2,4-di-tert. amylphenoxy acetyl chloride to form the final product which was found to have a melting point of 133 to 135° C.

Compounds 6, 7 and 8 were made in the same way as compound 5 using, respectively, 2,5-dichloroaniline, 2,4,6-trichloroaniline and 2,4,6-tribromoaniline in place of the 2,4-dichloroaniline.

Compound 9 was prepared by the same procedure as compound 2 using  $\beta$ -2,4-di-tert. amylphenoxy propionyl chloride (Weissberger et al. U. S. application Serial No. 83,762) instead of benzoyl chloride. It had a melting point of 220-222° C.

Compound 10 was prepared by the same procedure as compound 1 using  $\beta$ -2,4-di-tert. amylphenoxy propionyl chloride instead of benzoyl chloride. It had a melting point of 225-227° C.

Compound 11 was prepared by condensing 1-(2',5'-dichlorophenyl)-3-amino-5-pyrazolone with 4'-tert. amyl-3-phenoxybenzoyl chloride (Weissberger et al. application Serial No. 83,762). It had a melting point of 110-112° C.

Compound 12 was prepared in the same way as compound 11, using 1-(2',4',6'-tribromophenyl)-3-amino-5-pyrazolone instead of the 2,5-dichlorophenyl derivative. It had a melting point of 270-272° C.

Certain of our compounds may be used in developing solutions containing a primary aromatic amino developing agent. Compounds 1 to 4 may be used in this way. The following example illustrates a developing solution which may be used with the compounds of our invention.

## A.

|                                 | Grams |
|---------------------------------|-------|
| p-Amino diethyl aniline sulfate | 2     |
| Sodium sulfite (anhydrous)      | 5     |
| Sodium carbonate (anhydrous)    | 20    |
| Potassium bromide               | 2     |
| Water to 1 liter.               |       |

## B.

|                                                       |       |
|-------------------------------------------------------|-------|
| 1-(2',4',6'-trichlorophenyl)-3-benzamido-5-pyrazolone | grams |
| 2                                                     |       |
| Sodium hydroxide (2% solution)                        | cc    |
| 50                                                    |       |

For use, B is added to A.

Certain of our couplers may be incorporated in sensitive silver halide emulsion layers as described in Mannes and Godowsky U. S. Patent 2,304,940 or Jelley and Vittum U. S. Patent 2,322,027. Compounds 5 to 12 may be used in this way. For example, compound 7 may be incorporated in a silver halide emulsion as described in Example 1 of Jelley and Vittum U. S. Patent 2,322,027. When used in this way, the exposed emulsion layer may be developed in a solution having the composition of Part A of the developing solution described above.

The aromatic amino developing agents used with the coupler compounds of our invention include the mono-, di- and tri-amino aryl compounds and their derivatives formed by substitution in the amino group as well as in the ring such as alkyl phenylene diamines and alkyl toluylene diamines. These compounds are usually used in the salt form such as the hydrochloride or the sulfate which are more stable than the amines themselves. Suitable compounds are di-

ethyl-p-phenylene diamine hydrochloride, monoethyl-p-phenylene diamine hydrochloride, di-methyl-p-phenylene diamine hydrochloride, di-methyl-p-phenylene sulfate and 2-amino-5-diethyl amino toluene sulfate. The p-amino phenols and their substitution products may also be used where the amino group is unsubstituted. All of these compounds have an unsubstituted amino group which enables the oxidation products of the developer to couple with the color-forming compounds to form a dye image.

Our development process may be employed for the production by colored photographic images in layers of gelatin or other carrier for the silver halide such as collodion, organic esters of cellulose or synthetic resins. The support for the emulsion may be a transparent material such as glass, cellulose ester or a non-transparent reflecting material such as paper or an opaque cellulose ester. The emulsion may be coated as a single layer on the support or as superposed layers on one or both sides of the support. The superposed layers may be differentially sensitized to form natural color photographic images in the well-known manner. For example, in a multi-layer material sensitized to red, green and blue light, respectively, our couplers would ordinarily be used in the green-sensitive emulsion layer to form the magenta image.

Dyes formed from the couplers of our invention have an absorption maximum in the green spectral region which is shifted toward the red by about 50 to 200 millimicrons as compared with dyes from corresponding couplers with a simple 1-phenyl or 1-chlorophenyl substituent. At the same time, there is little or no increase in absorption in the blue and red regions of the spectrum.

We claim:

1. The method of producing a magenta-colored image in a silver halide emulsion layer which comprises exposing said layer and developing it with a primary aromatic amino developing agent in the presence of a 1-phenyl-3-acylamino-5-pyrazolone coupler compound having at least two halogen substituents on the 1-phenyl radical.

2. The method of producing a magenta-colored image in a silver halide emulsion layer which comprises exposing said layer and developing it with a primary aromatic amino developing agent in the presence of a coupler compound having the formula:



60 where COR is an acyl radical.

3. The method of producing a magenta-colored image in a silver halide emulsion layer which comprises exposing said layer and developing it with a primary aromatic amino developing agent in the presence of a coupler compound having the formula:



75 where COR is an acyl radical.

4. The method of producing a magenta-colored image in a silver halide emulsion layer which comprises exposing said layer and developing it with a primary aromatic amino developing agent in the presence of a coupler compound having the formula:



5. The method of producing a magenta-colored image in a silver halide emulsion layer which comprises exposing said layer and developing it with a primary aromatic amino developing agent in the presence of a coupler compound having the formula:



6. A photographic emulsion for forming a magenta-colored image comprising a silver halide emulsion having incorporated therein a 1-phenyl-3 - acylamino - 5 - pyrazolone coupler compound having at least two halogen substituents on the 1-phenyl radical.

7. A photographic emulsion for forming a magenta-colored image comprising a silver halide emulsion having incorporated therein a coupler compound having the formula:



where COR is an acyl radical.

8. A photographic emulsion for forming a magenta-colored image comprising a silver halide emulsion having incorporated therein a coupler compound having the formula:

ide emulsion having incorporated therein a coupler compound having the formula:



where COR is an acyl radical.

9. A photographic emulsion for forming a magenta-colored image comprising a silver halide emulsion having incorporated therein a coupler compound having the formula:



10. A photographic emulsion for forming a magenta-colored image comprising a silver halide emulsion having incorporated therein a coupler compound having the formula:



ANTHONY LORIA.  
ARNOLD WEISSBERGER.  
PAUL W. VITTM.

#### REFERENCES CITED

The following references are of record in the file of this patent:

#### UNITED STATES PATENTS

| Number    | Name                 | Date           |
|-----------|----------------------|----------------|
| 2,213,986 | Kendall et al. ----- | Sept. 10, 1940 |
| 2,343,702 | Porter et al. -----  | Mar. 7, 1944   |
| 2,369,489 | Porter et al. -----  | Feb. 13, 1945  |

#### FOREIGN PATENTS

| Number  | Country      | Date          |
|---------|--------------|---------------|
| 836,144 | France ----- | Jan. 11, 1939 |